

No. 839,374.

PATENTED DEC. 25, 1906.

W. L. R. EMMET & W. S. CLARK.  
INSULATED ELECTRIC CONDUCTOR.  
APPLICATION FILED NOV. 9, 1901.

Fig.1.



Fig.2.



Fig.3.



Witnesses:

Marcus D. Byng.  
Benjamin P. Vice.

Inventors

William LeRoy Emmet,  
Wallace S. Clark,  
by Albert G. Davis, Atty.

# UNITED STATES PATENT OFFICE.

WILLIAM L. R. EMMET AND WALLACE S. CLARK, OF SCHENECTADY,  
NEW YORK, ASSIGNORS TO GENERAL ELECTRIC COMPANY, A COR-  
PORATION OF NEW YORK.

## INSULATED ELECTRIC CONDUCTOR.

No. 839,874.

Specification of Letters Patent.

Patented Dec. 25, 1906.

Application filed November 9, 1901. Serial No. 81,658.

*To all whom it may concern:*

Be it known that we, WILLIAM LE ROY EMMET and WALLACE S. CLARK, citizens of the United States, residing at Schenectady, county of Schenectady, State of New York, have invented certain new and useful Improvements in Insulated Electric Conductors, of which the following is a specification.

This invention relates to insulated electric conductors, with a view to providing a conductor or cable having high insulating properties, being thoroughly moisture-proof and cheap to manufacture.

It relates to an improvement upon the type of conductor described in Patent No. 666,003, granted to William Le R. Emmet January 15, 1901. In said patent is described a form of conductor in which multiple layers of flexible fabric coated with an insulating-varnish composed principally of linseed-oil were wound over a conductor, successive layers being coated a number of times with the insulating-varnish. Such a form of construction, although extremely effective for insulating purposes, is slow in manufacture by reason of the time required for the films of varnish to dry and harden. We promote a much greater expedition in manufacture by preparing the fabric as a preliminary stage of the manufacture and carrying the conductor or cable, after each layer of the fabric is applied, through a bath containing a viscous insulating compound which will effectively seal the joints of the winding and provide a soft yielding film between the several layers, which will permit slipping of one layer upon another when the conductor or cable is bent, and thereby prevent fracture of the insulation, enabling it to meet all the requirements of practical service without impairing the insulation at some point where a bend is necessarily made, and thereby impairing the insulation of the entire cable.

We wind as many layers of the coated fabric upon a core as required for the potential to which the cable is to be subjected, a cable having a dozen layers being capable of withstanding twenty thousand volts and upward. In applying the coated fabric to the core it is wound in a spiral with butt-joints, the cable being then passed through a bath of the viscous compound and another spiral winding applied in a manner similar to

the first but with the joints lapped. In the same way the cable is built up of a number of superposed layers having overlapping joints with a viscous substance intervening between the several layers, permitting it to be bent or distorted with impunity and being proof against the infiltration of moisture and retaining for an indefinite length of time its high insulating properties. After the final covering has been applied an armor of lead or other suitable material may be applied over the outside to prevent abrasion.

In the accompanying drawings is illustrated a conductor embodying our improvements, Figure 1 being a side elevation with successive layers of the insulating fabric partially unwound to show their relative arrangement. Fig. 2 is a cross-section of a cable embodying our improvements, and Fig. 3 is a section of the varnished fabric.

1 represents the insulated conductor, which may be a single wire or a group of wires. On this are laid a number of windings, as 2 3, of muslin, paper, or other vegetable or organic flexible fabric, each layer being coated on both sides with an insulating-varnish containing an excess of an oxidizable oil. The composition of this varnish may be varied in practice; but we find excellent results from a mixture of about eighty parts of boiled linseed-oil and twenty of rosin, which may be thinned for application by a solvent, such as benzine. The paper may be given more than one coat. In practice we find that two coats give superior results. Each layer is wound spirally about the conductor, so as to have the edges abut against one another, thus forming a close spiral. The covered conductor is then led through a bath containing a compound of rosin, seventy-five per cent., and transil-oil or rectified petroleum, twenty-five per cent. The process is repeated for as many layers as deemed necessary for the voltages the conductor is to withstand. Six are shown, by way of example, in the drawing Fig. 2. The rosin compound is heated to drive off moisture and air from the covered conductor and permit an effective sealing of the joints by the viscous compound. The successive layers are arranged with overlapping joints to more effectively seal the inner layers against infiltration of moisture, and the joints are

sealed to effectively cover the ends of any protruding fibers of the fabric with a water-proof covering, so as to prevent a gradual soaking in of moisture through such fibers to the body of the fabric. Thus by means of our construction we provide a covering in which there is an absolute certainty of no short air-paths existing between the conductor and the outside covering, and any leakage-path which by any possibility could exist would be so long that it would require an extraordinary potential to break it down.

The viscous compound is particularly advantageous in permitting a rapid manufacture of the conductor. By covering the joints with the oil compound, as described in the prior patent above referred to, the process is necessarily much slower than our present process. The latter, moreover, has the advantage of supplying between the layers a yielding compound which renders the cable much more flexible and permitting the layers to slide one upon another when the cable is bent, thereby preventing cracks in the insulation. Besides, the compound seals the joints as well as the spaces between the several layers.

We do not confine ourselves to the viscous medium described, as others may be used with greater or lesser advantage. Asphalt, very soft ozocerite, a mixture of rosin and rosin-oil, rosin and petroleum-oil, non-drying varnishes, or any suitable plastic insulation which will not act injuriously on the films of varnish, may be employed, the essential feature being the application of a film of plastic

insulation to the joints and between the layers of a varnished fabric.

What we claim as new, and desire to secure by Letters Patent of the United States, is— 40

1. An insulated electric conductor, covered with a plurality of layers of preliminary varnished and hardened fabric, and a homogeneous layer of permanently-viscous insulating material forming a continuous covering 45 for the layers of fabric.

2. An insulated electric conductor, covered with a plurality of layers of flexible fabric preliminarily coated on both sides with a tough, oxidized film of a vegetable oil, and a 50 layer of permanently-viscous insulating compound, forming a continuous covering for the layers of fabric and applied directly thereto.

3. An insulated electric conductor, covered with a plurality of layers of fabric, each 55 layer preliminarily coated on both sides with a hard, dry, tough film of an insulating compound containing oxidized oil in excess and wound helically on the conductor with the edges in contact, successive layers having 60 overlapping joints, and a homogeneous layer of permanently-viscous insulating material, forming a continuous covering for the layers of fabric.

In witness whereof we have hereunto set 65 our hands this 7 day of November, 1901.

WILLIAM L. R. EMMET.  
WALLACE S. CLARK.

Witnesses:

BENJAMIN B. HULL,  
HELEN ORFORD.